

Nov. 30, 1926.

1,609,033

T. W. MORSE

TRANSFER SHEET

Filed May 23, 1925



Fig 1



Fig 2

INVENTOR.  
Tally W. Morse  
BY  
Lyman E. Dodge  
ATTORNEY

Patented Nov. 30, 1926.

1,609,033

# UNITED STATES PATENT OFFICE.

TALLY W. MORSE, OF NEW YORK, N. Y.

## TRANSFER SHEET.

Application filed May 23, 1925. Serial No. 32,278.

This invention relates to a process for making transfer sheets and an ink for use in the process.

Heretofore transfer sheets have been made by a process which included an ink which by reason of its character had to be kept quite a little above the ordinary temperature in order to work properly. With such an ink and with the usual processes a comparatively small number of transfer sheets may be formed per hour, consequently they are comparatively costly.

Heretofore the difficulties of the process wherein the ink must be warmed have been sought to be overcome, but in so doing resort has been had to such coloring matters as aniline dyes, which when transferred on to such material as silk become indelible and cannot be washed out.

Applicant has as an object a process and an ink therefor by which transfer sheets may be printed cold and the transfer made on to the material is fugitive, when washed as in ordinary practice.

In describing the invention in detail and a particular product made by the use of the process, reference is had to the accompanying drawing, wherein I have illustrated a particular product and wherein like characters of reference designate corresponding parts throughout the several views, and in which:

Figure 1 illustrates a transfer sheet with a design in the plurality of colors thereon; Fig. 2 illustrates a transfer sheet with a design in one color thereon.

In order to carry out the process applicant has devised a printing composition, called, an ink.

The ink used by applicant is made preferably in the following manner. Ordinary rosin of commerce is heated in any suitable or appropriate way until it will flow freely. In a separate receptacle mineral paraffine, the ordinary paraffine of commerce, is heated until it will flow freely. The two, rosin and paraffine, are then mixed, by pouring one into the other, with constant stirring. In addition to the rosin and paraffine, cocoa butter and mutton tallow are melted together in a receptacle until they will flow freely and are then mixed with the mixed rosin and paraffine by pouring therein with constant stirring.

The mixture resulting from the above de-

scribed operations is then ground either by hand or in some such device as a suitable type of power paint mill and to it is added preferably as the grinding proceeds, such quantity of coloring matter as will give the desired color and shade to the transfer design when impressed upon the desired material.

The coloring matter used by applicant is a most important element of the invention. Applicant has found that for his purposes a mineral coloring matter is most appropriate, because the composition of his ink is such that although the ordinary handling of his transfer sheets when dry will not smudge the design and damp fingers rubbed thereon will not smudge the design, nevertheless, a vigorous washing of the material to which the design is transferred will remove the ink from the material. Applicant has found that if a mineral coloring matter, that is, one which does not combine with the material, to in effect dye it, is used, it being merely held mechanically by the ink on the material, it is also removed, by washing, so that it is fugitive.

After properly grinding the mixture, I adjust the viscosity so that it will work properly with the particular type of press and ink rollers used. I do this by adding rosin made fluid by heat until by trial I reach the exact viscosity desired.

The quantities used in making my ink are about as follows:

|               | Ounces. |
|---------------|---------|
| Mutton tallow | 1 90    |
| Cocoa butter  | 1       |
| Paraffine     | 4       |
| Rosin         | 6       |

Additional rosin, a sufficient quantity. Mineral pigment, a sufficient quantity.

Any desired mineral pigment may be used that will give the desired color.

If what is technically known as "offsetting" occurs the quantity of rosin may be slightly increased, and in general the viscosity of the ink will be regulated by the type of roller present on the press upon which the ink is used.

The ink made as hereinbefore described is usable upon ordinary plate presses. The ink being used to fill the usual font and the printing of the transfer sheets being accomplished as ordinary printing.

In Fig. 1, I have illustrated a five pointed

star on a sheet 1. The points 2 and 3 of the star are colored respectively, yellow and blue. In Fig. 2, I have illustrated a five pointed star in outline on sheet 4 the bounding lines all being in one color, preferably blue. For the yellow, I preferably use chrome yellow and for blue, ultramarine.

In use the transfer sheet is applied, after 10 drying, in reverse on the material to which the design is to be applied and a hot roller or sad iron is applied thereto, whereupon the design will be transferred to the material, reproducing the color or colors on the transfer sheet.

15 Although I have particularly described my process and products resulting from my process, nevertheless, I desire to have it understood that the forms selected are merely 20 illustrative but do not exhaust the possible expressions of the idea of means underlying my invention.

What I claim as new and desire to secure by Letters Patent of the United States, is:

1. The process of producing water-fugitive 25 designs on textiles, fabrics and the like,

consisting in printing upon a base, a design or configuration in water-fugitive heat-releasable material embodying a mineral pigment, said material being at ordinary atmospheric temperatures, whereby the design 30 may be transferred to a fabric material by the application of heat and may be removed therefrom by the application of water.

2. The process of producing water-fugitive 35 designs on textiles, fabrics and the like, comprising the printing upon a suitable base at ordinary temperature a design or configuration in a medium embodying paraffine, rosin, cocoa butter, mutton tallow and 40 mineral coloring matter, whereby the design may be transferred to a fabric material by the application of heat and may be removed therefrom by the application of water.

3. A transfer paper or base having a design or configuration thereon in a medium 45 embodying paraffine, rosin, cocoa butter, mutton tallow and a mineral coloring matter.

TALLY W. MORSE.